

## 1

3,234,036

**PROCESS FOR THE MANUFACTURE OF SHAPED ARTICLES FROM REGENERATED CELLULOSE**  
Hanswilli von Brachel, Cologne-Sulz, and Heinz Dietrich Jordan, Leverkusen, Germany, assignors to Farbenfabriken Bayer Aktiengesellschaft, Leverkusen, Germany, a corporation of Germany  
No Drawing. Filed Oct. 24, 1962, Ser. No. 232,891  
Claims priority, application Germany, Nov. 2, 1961,  
F 35,264

4 Claims. (Cl. 106—165)

The subject of the present invention is a process for the production of fibres, threads or films from regenerated cellulose, which are characterised by low swelling and high strength.

The higher demands recently made on such products in regard to their use for textile and technical purposes, in particular for their use in tyre cords had led to a search for methods of suitably modifying the customary viscose process to obtain material of the desired properties.

Thus, methods are known in which so-called modifiers are added to the viscose or to the spinning bath in order to retard the xanthogenate decomposition and to reduce the gel swelling value, which frequently improves the properties of the spun threads. At the same time, the other spinning conditions also have had to be adapted to these altered conditions, for example it may be necessary to use higher concentrations of zinc sulphate and lower concentrations of sulphuric acid in the precipitating bath or to use a separate second bath in which the necessary stretching of the resulting threads may be carried out.

Compounds which are capable of producing the desired effects include numerous mono and polyamines and their alkoxylated products and polyglycol ethers of various compositions or mixtures of the two classes of substances.

It is an object of the present invention to enable threads of low swelling and increased tensile strength and increased elongation to be produced by the viscose process. A further object of the invention consists in providing novel additives for the viscose in the viscose spinning process. Further objects of the invention will be clear from the following description and examples.

It has now been found that to achieve the above objects it is particularly advantageous to use polyether sulphonium compounds which are soluble at least to the extent of 0.1% in 5% sodium hydroxide solution and preferably have a molecular weight between 300 and 20,000. It is preferred to use those polyether sulphonium compounds in which the cation contains at least one ether oxygen atom or one sulphonium group for every 4 carbon atoms. The polyether sulphonium compounds are prepared by ternating polyether thioethers, the latter being obtainable by various methods. For example, the thioethers used as starting material may be prepared by oxalkylating mono-, di- or polymercaptans or mono-, di- or polythioether alcohols, by condensing di- or polyhalogen alkyl-ethers with alkali metal sulphides or mono-, di- and polymercaptans, by copolymerisation of alkylene sulphides with alkylene oxides or by mixed condensation of polyalkylene glycols with  $\beta$ - or  $\gamma$ -hydroxy-alkyl sulphides. It is particularly advantageous to use the polyether thioethers which are described in French patent specification 1,201,171. The ternating of these polyether thioethers may be carried out with a large variety of alkylating agents, for example methyl iodide, allyl bromide, benzyl chloride, dimethyl sulphate, diethyl sulphate, triethyl phosphate, methylmethane sulphonate, methyl-p-toluene-sulphonate or other alkylating

## 2

agents such as those described in German patent specification 880,485 or in German Auslegeschrift 1,062,014.

The polyether sulphonium compounds used in accordance with the invention have the particular advantage that they are mixed homogeneously more easily with the viscose than the additive hitherto proposed, so that they are more effective. This also makes it possible to vary the other spinning conditions, particularly the nature of the viscose and the precipitating bath within wider limits than is possible with the use of many other modifiers, so that for example even when spinning ordinary commercial viscose in acid precipitating baths of the usual composition (i.e., baths having a higher concentration of sulphuric acid and sodium sulphate and lower concentration of zinc sulphate than indicated for the above-mentioned process) followed by stretching in air after the ordinary winding or centrifuging processes, a marked improvement in the qualities of the fibres may be obtained.

20 The compounds that may be used in accordance with the invention may very conveniently be applied by means of the dosing process used in spin dyeing, because when they have been injected in the form of their aqueous or alkaline solution into the main stream of the viscose and have passed through the mixing apparatus customarily provided in such plants, they are already uniformly distributed as required.

By this method, smaller proportions of modified viscous may be worked up without the necessity of having afterwards to clean extensive pipe systems, which is normally a very time-consuming process. Production is therefore more adaptable, for example because it is easier to transfer from one fibre type to another.

30 The substances incorporated in the viscose in accordance with the present invention can not only retard coagulation and thereby influence the formation of the threads in the viscose and in the spinning bath, but owing to their pronounced cationic character and their surface activity they can produce other effects which are advantageous for the spinning process. Examples of these include: improved filtering of the viscose, improved drawing of the threads, reduced tendency to block spinnerets and form incrustations, clarification of the spinning bath and the like. These features illustrate further advantages of 40 these substances compared with the non-ionic polyalkylene oxide compounds. In order to improve the spinning process in this sense, it has been customary for a long time to add so-called spinning oils to the viscose. These are surface active products of various types. The use of 45 these spinning oils becomes superfluous in the method according to the invention.

The above described polyether sulphonium compounds may be added to the viscose in quantities which vary depending on the effect desired on the fibres and 50 with the other conditions, the quantities varying between 0.1 and 4%, preferably 0.1 and 0.6% by weight.

55 The dosing process may be carried out with the usual apparatus without any additional equipment.

As already mentioned above, the production of fibres, 60 threads and films of improved mechanical properties by the process according to the invention is not limited to particular compositions of viscose and of the spinning bath.

65 However, the precipitating baths preferably contain at least 3% by weight of zinc sulphate. The stretching of the spun threads, which is necessary in order to obtain good textile properties, may be carried out by known methods either in the spinning bath or in air or in special stretching baths.

70 The fibres and threads obtained with the use of the above mentioned viscose additives are distinguished from those prepared without the use of these additives by

having a flattened cross-section, e.g., kidney shaped, reduced swelling and increased dry tensile strength and wet tensile strength without reduced elongation at break.

The invention is further disclosed in the following examples which are illustrative but not limitative thereof.

*Example 1*

A viscose containing 7.5% cellulose and 5.0% total alkali and to which 2.25 g. of the compound described below has been added per kg. of viscose was spun at a degree of maturity corresponding to a salt point 8 from a spinneret having 48 apertures of 90 $\mu$  diameter into an acid precipitating bath to form a thread of 180 total denier.

The bath contained 125 g./l. sulphuric acid, 250 g./l. sodium sulphate and 30 g./l. of zinc sulphate and the temperature of the bath was 45° C. After leaving the spinning bath, in which it had traversed 50 cm., the thread was stretched in air between 3 rollers by a total amount of 100%, the last roller having a draw-off speed of 36 m. per minute.

The material thus obtained was then collected in a spinning pot which revolved at the rate of 6000 revs. per minute and was then deacidified in the usual manner and treated and dried under tension.

When comparing the textile properties with those of a thread prepared from viscose without the addition of the above mentioned compound but otherwise by the same method as described above, the following differences were found:

The swelling value was reduced by 28%. The dry tensile strength was increased by 19% and the wet tensile strength was increased by 25% and the elongation in the dry and the wet state were increased by 3% and 3.6% respectively.

This shows that the above mentioned viscose additives can considerably improve the mechanical properties.

The polyether sulphonium compound used in this example was prepared as follows:

600 g. of polyethylene glycol having a molecular weight of 600, 200 g. of thiodiglycol and 8 g. phosphoric acid were heated in a current of CO<sub>2</sub> at 185° C. until the condensate had a hydroxyl number of 42. Steam was then blown through the reaction product for 4 hours at 120° C. and 15 mm. Hg and the product was then dried for one hour at 120° C. and 15 mm. Hg and then slowly treated with 220 g. dimethylsulphate at 95° C. When the exothermic reaction had ceased, the product was heated for one more hour at 95°.

*Example 2*

2 g. of the compound described below were added per kg. of viscose to a viscose with 7.2% cellulose and 4.8% alkali. The process was then continued as described in Example 1 except that a precipitating bath composed of 100 g./l. sulphuric acid, 230 g./l. sodium sulphate and 40 g./l. zinc sulphate at a temperature of 50° C. was used and only 2 rollers were used for stretching the thread by 100%.

On determining the textile data and comparing them

with those found in threads produced from viscose without additives, it was found that the swelling value was reduced by 35% and the dry tensile strength and wet tear strength was increased by 17% and 21% respectively.

The polyether polysulphonium compound was prepared as in Example 1 except that instead of using polyethylene glycol with molecular weight 600, an equivalent quantity of oxyethylated tripropylene glycol with molecular weight 1200 was used.

*Example 3*

Observing the same reaction conditions as in Example 1 and using 1.5 g. per kg. of viscose of the compound described below, the threads differed from those prepared from unmodified viscose as shown below:

Reduction in swelling: 24%; increase in dry tensile strength: 20%; increase in wet strength: 22%.

The polyether polysulphonium compound used was prepared as in Example 1 except that the polyether thioether had a hydroxyl number of 14 corresponding to a molecular weight of 8000.

We claim:

1. Viscose spinning solution which contains 0.1-4.0% by weight of a polyether sulphonium compound containing one member of the group consisting of a sulphonium group for every four carbon atoms in the polymer chain, an ether group for every four carbon atoms in the polymer chain, and a sulphonium group plus ether oxygen for every four carbon atoms in the polymer chain, said compound being soluble at least to the extent of 0.1% in a 5% aqueous sodium hydroxide solution and having a molecular weight between 300 and 20,000.

2. Viscose spinning solution according to claim 1 which contains a polyether sulphonium compound having in its cation at least one ether oxygen atom for every four carbon atoms.

3. Viscose spinning solution according to claim 1 which contains a polyether sulphonium compound having in its cation at least one sulphonium group for every four carbon atoms.

4. Viscose spinning solution containing 0.1 to 4.0 weight percent of the viscose of a polyether sulphonium compound having an average molecular weight of from 300 to 20,000 and at least one ether oxygen and sulphonium group for every four carbon atoms, said polyether sulphonium compound being soluble at least to an extent of 0.1% in a 5 weight percent aqueous sodium hydroxide solution.

References Cited by the Examiner

UNITED STATES PATENTS

3,116,353 12/1963 Brower \_\_\_\_\_ 106-165  
3,151,194 9/1964 Van Doorn et al. \_\_\_ 106-165

FOREIGN PATENTS

1,035,850 8/1959 Germany.  
478,774 1/1938 Great Britain.

MORRIS LIEBMAN, Primary Examiner.